

## UNITED STATES PATENT OFFICE

2,188,073

## TEXTILE PRINTING LACQUER

Edmond H. Bucy, Stamford, Conn., assignor to  
 Atlas Powder Company, Wilmington, Del., a  
 corporation of Delaware

No Drawing. Application June 10, 1938,  
 Serial No. 213,097

6 Claims. (Cl. 91—68)

This invention relates to printing lacquers for printing textiles, such as rayon, silk, satin, cotton, and the like, and more particularly to lacquers for solid color, contrast printing of textiles by means of an engraved roll, and to the printed textile.

In the printing of textiles with solid color lacquers, great difficulty has been encountered with "crocking" or "dry marking off" of the printed pattern, particularly where the color of the lacquer is in sharp contrast with the color of the fabric. "Crocking" or "dry marking off" is the tendency of the printing to rub off, a tendency which is aggravated with solid, contrasting colors where the lacquer print should be in sufficient amount to give good coverage. Furthermore, the solid color lacquers when applied to textiles have tended to stiffen the printed portion of the fabric so appreciably as to spoil its feel or hand.

An object of the present invention is the production of a solid color lacquer for printing textiles which overcomes the foregoing difficulties.

Another object of the invention is the production of a textile having a solid color lacquer design printed thereon, the printed portion of the textile having a softness of feel or hand of about that of the unprinted portion.

Other objects of the invention will hereinafter more fully appear.

I have found that solid printing colors having a solids content consisting essentially of a cellulose derivative comprising at least 50% ethyl cellulose, shellac, a straight chain dibasic acid-polyhydric alcohol resinous reaction product, a plasticizer, and a pigment, are highly valuable in that they may be roll printed on fabrics in quantities sufficient to cover well, and yet do not "crock" or "dry mark off." The combination of ethyl cellulose, shellac and straight chain dibasic acid-polyhydric alcohol resinous reaction product appears to give the solid content of the lacquer the quality of adhesion to the fiber of the cloth and the plasticity of the resin employed, plus the added plasticizer, renders the print highly flexible, thereby maintaining the desired feel or hand of the fabric.

Preferably, the ethyl cellulose employed in the printing lacquer is high-viscosity ethyl cellulose of viscosity of at least 5 seconds as determined by the falling ball method ( $\frac{1}{8}$ " steel ball, 10' drop) in a 16-ounce (12.2%) solution of ethyl cellulose in 80:20 toluene: ethyl alcohol at 25° C. The employment of ethyl cellulose of less than 44% ethoxy content is highly advantageous, as such ethyl cellulose is of low solubility in dry

cleaning solvents such as carbon tetrachloride. Where, in addition to ethyl cellulose, another cellulose derivative is employed, it may be a cellulose ether such as benzyl, propyl or amyl cellulose, or a cellulose ester such as the nitrate, acetate, 5 aceto propionate, or aceto butyrate.

The resinous reaction products employed are the resinous esterification products of the straight chain dibasic acids, such as adipic, sebacic, azelaic, suberic and pimelic, and poly- 10 hydric alcohols, such as glycerine and the glycols. Resins of this type are characterized by their plasticity and may be obtained under the trade name "Paraplex."

As the plasticizer, there may be employed di- 15 butyl phthalate, diethyl phthalate, tricresyl phosphate, and other like plasticizers which do not impart odor to the print.

It is important that the resinous reaction product and the plasticizer be employed in an amount sufficient to give the print extreme softness so that the desired feel or hand of the fabric will not be destroyed. Generally, the resinous reaction product and the plasticizer are each present in an amount greater than the shellac and the 25 resinous reaction product is present in an amount greater than the cellulose derivative. Such a print lacquer, if applied to a solid, non-absorptive surface such as steel, would remain permanently soft and tacky and would lack adhesion. When applied to textiles, however, the print lacquer dries readily and adheres to the fabric, and due to the high plasticizer content and the plasticity of the resin employed, the 30 flexibility of the fabric is maintained. 35

The coloring material employed may be any suitable pigment. Colloidal dispersed pigments of the desired color have been found to insure maximum fastness and best color values and are generally preferred. By the term "pigment" I 40 mean to include lakes and toners and to exclude soluble dyestuffs which are undesirable for solid color printing lacquers.

The solvents in which the solids are carried preferably consist, for example, of a preponderance of highly volatile, rapidly evaporating, organic solvents, such as toluol, alcohol, ethyl acetate, acetone, or of any other solvents which have a relatively low boiling point and vapor pressure. Smaller amounts of less volatile, more slowly evaporable solvents, such as butyl acetate, xylol, methyl isobutyl ketone, butyl alcohol, and the like, may be used along with the more highly volatile solvents with advantage. 45 50 55

A non-limiting example of a printing color lacquer of the present invention is as follows:

|                                                                        | Per cent<br>by weight |
|------------------------------------------------------------------------|-----------------------|
| 5 Toluidine toner                                                      | 4.75                  |
| 1/2 sec. nitrocotton                                                   | 3.25                  |
| Dibutyl phthalate                                                      | 5.5                   |
| High viscosity ethyl cellulose                                         | 4.0                   |
| Paraplex RG-2                                                          | 8.75                  |
| 10 Montan wax                                                          | 0.5                   |
| Shellac solution (6 lbs. shellac cut into one<br>gallon ethyl alcohol) | 4.5                   |
| Butyl acetate                                                          | 12.25                 |
| Toluol                                                                 | 43.5                  |
| 15 Ethyl alcohol                                                       | 1.5                   |
| Petroleum naphtha                                                      | 2.5                   |
| Ethyl acetate                                                          | 9.0                   |

In the preparation of the printing lacquer of the foregoing example, the red pigment, 1/2 sec. nitrocotton and dibutyl phthalate were dispersed in a Banbury machine and thereafter admixed with the other ingredients. The resulting printing lacquer had a viscosity of about 500 centipoises and gave excellent results in contrast printing on rayon textiles using both blotch and line patterns. In the printing operation the printing lacquer was fed directly on to a doctor blade, which applied the lacquer to the engraved portion of an engraved copper roll. By passing the textile about another roll in rolling contact with the engraved roll, the lacquer was cleanly transferred from the engraved portion of the roll to the fabric. The fabric, after printing, was run through a tunnel dryer and after drying, the surface of the printing was neither soft nor tacky and yet the pattern was highly flexible and did not materially change the hand or feel of the fabric.

It is to be understood that the foregoing example is merely for purpose of illustrating the invention and is not to be taken as limiting. The pigment need not be separately dispersed but may be admixed with the other solids in a colloid or other mixing device. The cellulose derivative content may consist entirely of ethyl cellulose or the nitrocotton portion may be replaced with other suitable cellulose derivatives, it merely being essential that the cellulose derivative comprise at least 50% ethyl cellulose. Other plasticizers, resinous reaction products, shellac solutions and solvents may be employed in varying proportions so long as the print dries with the required adhesion to the fabric and the desired flexibility. Accordingly, the invention is not to be considered as limited by the foregoing example but includes within its purview any printing lacquer falling within either the terms or the spirit of the appended claims.

What I claim is as follows:

1. A printing lacquer for textiles, said lacquer having a solid content consisting essentially of cellulose derivative comprising at least 50% by weight of ethyl cellulose, a straight chain dibasic acid-polyhydric alcohol resinous reaction product, shellac, a plasticizer and a pigment. 5

2. A printing lacquer for textiles, said lacquer having a solid content consisting essentially of cellulose derivative comprising at least 50% by weight of ethyl cellulose having less than 44% 10 ethoxy content, a straight chain dibasic acid-polyhydric alcohol resinous reaction product, shellac, a plasticizer, and a pigment.

3. A printing lacquer for textiles having a solid content consisting essentially of cellulose derivative comprising at least 50% by weight of ethyl cellulose, a straight chain dibasic acid-polyhydric alcohol resinous reaction product, shellac, a plasticizer and a pigment, said lacquer being highly plasticized by having the resinous 20 reaction product and the plasticizer each present in an amount greater than the shellac and the resinous reaction product present in an amount greater than the cellulose derivative. 15

4. A textile having a portion thereof printed 25 with a composition to form a pattern of solid color in contrast with the color of the textile, said composition consisting essentially of cellulose derivative comprising at least 50% by weight of ethyl cellulose, a straight chain dibasic acid-polyhydric alcohol resinous reaction product, shellac, a plasticizer and a pigment. 30

5. A textile having a portion thereof printed with a composition to form a pattern of solid color in contrast with the color of the textile, said composition consisting essentially of cellulose derivative comprising at least 50% by weight of ethyl cellulose having less than 44% ethoxy content, a straight chain dibasic acid-polyhydric alcohol resinous reaction product, shellac, a plasticizer and a pigment. 40

6. A textile having a portion thereof printed with a composition to form a pattern of solid color in contrast with the color of the textile, said composition consisting essentially of cellulose derivative comprising at least 50% by weight of ethyl cellulose, a straight chain dibasic acid-polyhydric alcohol resinous reaction product, shellac, a plasticizer and a pigment, said composition having the resinous reaction product and the plasticizer each present in an amount greater than the shellac and the resinous reaction product present in an amount greater than the cellulose derivative to make the composition highly flexible and to give the printed portion of the textile 55 a softness of feel or hand of about that of the unprinted portion. 45

EDMOND H. BUCY.